

1

3,160,505

PROCESS FOR OBTAINING A PHOTOGRAPHIC IMAGE WITH IMPROVED IMAGE-TONE ACCORDING TO THE SILVER HALIDE DIFFUSION TRANSFER PROCESS

5 Jozef Frans Willems and Gerard Michiel Sevens, Wilrijk-Antwerp, and Louis Maria De Haes, Edegem-Antwerp, Belgium, assignors to Gevaert Photo-Producten N.V., Mortsel, Belgium, a Belgian company  
 No Drawing. Filed Nov. 6, 1961, Ser. No. 150,173  
 10 Claims priority, application Belgium Nov. 8, 1960  
 12 Claims. (Cl. 96—29)

This invention relates to the obtaining of black or bluish black image tones according to the photographic silver complex diffusion transfer process.

15 According to the known silver complex diffusion transfer processes, the principle of which is described in our British patent specifications 614,155 and 654,630, and in the German patent specification 887,733, a light-sensitive silver halide emulsion layer is exposed to an image 20 and then developed into contact with specially pretreated receiving material in the presence of a silver halide solvent. The exposed areas of the image are developed and do not undergo any further change. The undeveloped silver halide present in the unexposed areas is dissolved 25 by the silver halide solvent which is present either in the developer or in the receiving layer, transferred by diffusion into the receiving layer of the said receiving material and converted therein to metallic silver.

30 This conversion is promoted by the catalytic action of developing nuclei which are present. These nuclei normally consist of finely divided metal or metal sulfide. In this way, a positive image of the original is formed in the receiving layer and is apparent after separation of the latter from the emulsion layer.

35 Besides the classical development with an organic reducing agent in the presence of photochemical nuclei, metal sulfides such as zinc sulfide can also develop the transferred silver complex in the receiving layer into a silver sulfide image.

40 A disadvantage of the silver complex diffusion transfer process is the less agreeable brown image-tone of the obtained silver image in the finished image-receiving material.

45 It has now been found that a black or a bluish-black image-tone is obtained when using in the above-mentioned processes an imidazolidine-4-thione with the following general tautomeric formula:



50 wherein: each of  $R_1$ ,  $R_2$ ,  $R_3$ ,  $R_4$  represents a hydrogen atom, an alkyl radical, a substituted alkyl radical, an aryl radical or a substituted aryl radical, e.g., an alkaryl radical, or wherein  $R_1$  and  $R_2$  and also  $R_3$  and  $R_4$  two by two represent the atoms necessary for closing a saturated homocyclic ring or a substituted homocyclic ring.

55 Some compounds of this type which form the experiments appeared to be particularly suited for being applied

2

in the process according to the present invention, are identified below:



60 These compounds may be prepared according to known methods, e.g., those described by J. D. Christian, J. Org. Chem. 22 (1957), 398; Bucherer and Brandt, J. prakt. Chem. 140 (1934), 129; U.S. patent specifications 2,785,175 and 2,806,036, filed resp. December 15, 1955, and August 22, 1955, by J. D. Christian; C.A. 28, 4383, with reference to Science Repts., Tokyo Bunrika Daigaku, Sect. A; 2, 1-7 (1934), and C.A. 22, 2146.

65 The preparation for the greater part corresponds with the reaction of ketone cyanohydrines with ammonium sulfide.

70 The black-toning agent, according to this invention

may be present either in the developing bath, the image-receiving layer and/or in the silver halide emulsion layer. The image-receiving layer consists of gelatin containing in a dispersed form developing nuclei or a substance which can form developing nuclei with the diffused silver complexes.

The image-receiving layer contains per sq. m. preferably between 10 and 50 mg. of black-toning agent according to this invention.

When the black-toning agent according to this invention is added to the developing solution, the concentration of imidazolidine-4-thione derivative is preferably chosen between 0.05 g. and 5 g. per liter of developing solution.

If the black-toning agent is added to the silver halide emulsion layer, the concentration is preferably chosen between 0.02 g. and 1 gram per kg. of flowable emulsion.

The image-receiving layer is coated onto a support preferably a paper support. On the image-receiving layer a surface layer may be present as described in our Belgian Patent Numbers 609,394 and 609,395.

So the image receiving layer makes part of a "bi-pack" material. Onto the receiving layer a silver halide emulsion layer is coated. In the latter case the image receiving layer is hardened and the silver halide emulsion layer is either unhardened or little hardened.

After exposure, development and diffusion transfer, the exposed and developed silver halide emulsion layer is removed, e.g., by washing with warm water.

The developing substance used for developing the light-sensitive material, may be present either in the silver halide emulsion layer, in the alkaline developing solution, or in both. Mixtures of developing substances may also be considered.

The complexing agent forming a soluble complex with silver halide, preferably consists of sodium thiosulfate and may be added to the image-receiving layer as well as to the bath.

In order to avoid fogging in the exposed silver halide emulsion layers it is in many cases favorable to use a fog inhibiting compound. This fog inhibiting compound may be added either to the silver halide emulsion or to the bath. Besides the classically used fog inhibiting compounds, the imidazolidine-4-thiones are also suited for this purpose.

The following examples illustrate the invention without limiting, however, the scope thereof.

#### Example 1

A solution of 250 mg. of 2,2,5,5-tetramethyl imidazolidine-4-thione in 25 cm.<sup>3</sup> of ethanol is added to 1 kg. of gelatino silver chloro iodide emulsion ready for coating and containing 0.5% by weight of iodide. For preparing this emulsion 45 g. of silver nitrate have been used. This emulsion is sensitized to light of a wavelength from 500 to 570 m $\mu$  and is then coated onto a paper support in such a way that the obtained light-sensitive material comprises 1.5 g. of silver metal per sq. m.

After drying, this material is exposed in contact with an original to be reproduced, and then passed through a developing bath together with a paper provided with an image-receiving layer comprising a binding agent and developing nuclei. The developing bath comprises hydroquinone, 1-phenyl-3-pyrazolidone and sodium thiosulfate. On leaving the developing bath, both layers are squeezed into contact with each other and after a 10 to 20 seconds separated again. In the receiving-layer an image of the original is obtained with a markedly black image tone.

When, however, in a similar method no use is made of the aforesaid black-toning agent, images with a disagreeable yellow-brown image tone are obtained.

#### Example 2

400 cm.<sup>3</sup> of a 1% alcoholic solution of 2,2,5-trimethyl imidazolidine-4-thione are added to 1 kg. of a gelatino

silver chloride emulsion which has been prepared with 45 g. of silver nitrate.

This emulsion is sensitized to light of a wavelength from 500 to 570 m $\mu$  and coated onto a paper support in such a way that the obtained light-sensitive material contains 1.5 g. of metallic silver per sq. m. On proceeding as in Example 1, an image of the original is obtained.

In comparison with the image tone of a material containing however no black-toning agent as in Example 1, the image obtained is markedly black.

#### Example 3

A paper support is coated with an image-receiving layer from a suspension of the following composition:

|                                                                   |                  |                      |
|-------------------------------------------------------------------|------------------|----------------------|
| Water                                                             | cm. <sup>3</sup> | 274                  |
| Gelatin                                                           | g                | 10                   |
| Sodium thiosulfate                                                | g                | 12                   |
| Sodium sulfide                                                    | mol              | $7.7 \times 10^{-4}$ |
| Cobaltous nitrate 6 aq.                                           | mol              | $1.1 \times 10^{-3}$ |
| 1% alcoholic solution of 2,2,5,5-tetramethyl imidazoline-4-thione | cm. <sup>3</sup> | 17                   |

With 1 l. solution 13 sq. m. paper surface are covered.

This image-receiving layer in its turn is coated with a layer from a solution consisting of:

|                                                                                                 |                  |     |
|-------------------------------------------------------------------------------------------------|------------------|-----|
| 4% aqueous solution of carboxymethyl cellulose                                                  | cm. <sup>3</sup> | 45  |
| Water                                                                                           | cm. <sup>3</sup> | 155 |
| Sandozol (trade name for a sulfonated organic oil marketed by Sandoz, A.G., Basel, Switzerland) | g                | 0.6 |

A silver halide emulsion paper as used in Example 1, containing, however, no 2,2,5,5-tetramethyl imidazolidine-4-thione, after exposure in contact with an original to be reproduced is developed in a solution of the following composition:

|                         |                  |      |
|-------------------------|------------------|------|
| Water                   | cm. <sup>3</sup> | 1000 |
| Sodium sulfite          | g                | 75   |
| Sodium hydroxide        | g                | 10   |
| Potassium bromide       | g                | 1    |
| Hydroquinone            | g                | 16   |
| 1-phenyl-3-pyrazolidone | g                | 1    |

On leaving the developing bath the emulsion layer of this material is pressed into contact with the image-receiving layer of the above described material and separated therefrom after 10-20 sec.

In comparison with the image-tone of a material containing no black-toning agent, the image-tone obtained in this image-receiving layer shows a more neutral color.

#### Example 4

Example 3 is repeated after having substituted, however in the image-receiving layer a same amount of 2,2,5-trimethyl imidazolidine-4-thione for the 2,2,5,5-tetramethyl imidazolidine-4-thione.

In comparison with the image-tone of a material containing no black-toning agent, the image-tone obtained in this receiving layer shows a more neutral color.

#### Example 5

A silver halide emulsion layer as in Example 1, and an image-receiving layer as described in Example 3, none of these layers containing, however, 2,2,5,5-tetramethyl imidazolidine-4-thione, are treated as described in example 3, in a developing bath to which, however, 1 g. of 2,2,5,5-tetramethyl imidazolidine-4-thione has been added.

Both layers are then squeezed together for 10-20 sec. and then separated again. In the image-receiving layer

an image of the original is obtained which shows a more neutral black image-tone.

*Example 6*

Example 5 is repeated, substituting, however, 1 g. of 2,2,5-trimethyl imidazolidine-4-thione for the same amount of 2,2,5,5-tetramethyl imidazolidine-4-thione. In the image-receiving layer an image of the original is formed which shows a more neutral image-tone.

We claim:

1. A process for preparing a photographic image which comprises exposing a photographic silver halide emulsion layer to a subject, developing the emulsion layer, then transferring the silver halide by diffusion from the undeveloped areas of the emulsion layer to an image-receiving layer, the transfer being effected in contiguity with a silver halide solvent and at least one imidazolidine-4-thione compound having the following tautomeric formula:



wherein each of R<sub>1</sub>, R<sub>2</sub>, R<sub>3</sub>, and R<sub>4</sub> is a member selected from the group consisting of a hydrogen atom, and alkyl radical, and an aryl radical.

2. A process for preparing a photographic image which comprises exposing a photographic silver halide emulsion layer to a subject, developing the emulsion layer, then transferring the silver halide by diffusion from the undeveloped areas of the emulsion layer to an image-receiving layer, the transfer being effected in contiguity with a silver halide solvent and at least one imidazolidine-4-thione compound having the following tautomeric formula:



wherein each of X and Y are the necessary atoms to form a cycloaliphatic ring structure.

3. A process for preparing a photographic image which comprises exposing a photographic silver halide emulsion layer to a subject, developing the emulsion layer, then transferring the silver halide by diffusion from the undeveloped areas of the emulsion layer to an image-receiving layer, the transfer being effected in contiguity with a

silver halide solvent and at least one imidazolidine-4-thione compound having the following tautomeric formula:



10 wherein each of R<sub>1</sub> and R<sub>2</sub> is a member selected from the group consisting of a hydrogen atom, an alkyl radical, an aryl radical, and Y represents the atoms necessary to form a cycloaliphatic ring structure.

15 4. A process according to claim 1, wherein the imidazolidine-4-thione compound is present in the image-receiving material.

5. A process according to claim 2, wherein the imidazolidine-4-thione compound is present in the image-receiving material.

20 6. A process according to claim 3, wherein the imidazolidine-4-thione compound is present in the image-receiving material.

7. A process according to claim 1, wherein the imidazolidine-4-thione compound is present in the treating liquid.

25 8. A process according to claim 2, wherein the imidazolidine-4-thione compound is present in the treating liquid.

9. A process according to claim 3, wherein the imidazolidine-4-thione compound is present in the treating liquid.

30 10. A process according to claim 1, wherein the imidazolidine-4-thione compound is present in the light sensitive material.

35 11. A process according to claim 2, wherein the imidazolidine-4-thione compound is present in the light sensitive material.

12. A process according to claim 3, wherein the imidazolidine-4-thione compound is present in the light sensitive material.

40

References Cited in the file of this patent

UNITED STATES PATENTS

- |           |           |       |                |
|-----------|-----------|-------|----------------|
| 2,785,175 | Christian | ----- | Mar. 12, 1957  |
| 2,806,306 | Christian | ----- | Sept. 10, 1957 |
| 3,017,270 | Tregillus | ----- | Jan. 16, 1962  |

FOREIGN PATENTS

- |         |           |       |                |
|---------|-----------|-------|----------------|
| 595,695 | Belgium   | ----- | Feb. 1, 1961   |
| 217,057 | Australia | ----- | Sept. 11, 1961 |

OTHER REFERENCES

- Photo Science and Eng. 4. No. 5 (1960), pp. 257-263.  
Glafkides: Photographic Chemistry, 1, Fountain Press, London (1958), pp. 374-380.